

1

3,084,115

### METHOD OF VULCANIZING RUBBER

Wendell V. Smith, Nutley, N.J., and Verne G. Simpson, Scotia, N.Y., assignors to United States Rubber Company, New York, N.Y., a corporation of New Jersey  
No Drawing. Filed Jan. 16, 1959, Ser. No. 787,100

10 Claims. (Cl. 204—154)

This invention relates to the vulcanization of rubber by exposing it to ionizing radiation, and more particularly it relates to the acceleration or enhancement of such vulcanization by having certain acrylate, diacrylate or dimethacrylate compounds present in the rubber during such exposure to ionizing radiation.

It is known to the art that rubber may be at least partially if not completely vulcanized when placed in a field of ionizing radiation. There are, however, limitations on this process. First, after a certain amount of exposure to such radiations, rubber has been observed to degrade.

Second, the cost of subjecting a material to irradiation varies directly with the quantity of energy that must be used and this cost is quite high, such that presently, radiation vulcanization cannot compare in cost to ordinary heat vulcanization.

This invention shows that when small quantities of certain acrylate, diacrylate or dimethacrylate compounds are mixed in with natural rubber or SBR (i.e., styrene-butadiene rubber, formerly known as GR-S or Buna-S) the amount of ionizing radiation necessary to effect cure is substantially reduced as shown in the working examples and tabulated results below.

The term "ionizing radiation" is used here in its conventional sense as referring to radiation which when absorbed by matter produces ionization. Well known to the art as ionizing radiations are X-rays, gamma rays, high speed electrons, beta rays, and high speed protons, alpha particles and fast neutrons. Of these, X-rays, gam-

2

of at least about 8 electron volts. For more details of such energy, reference may be had to Table 10a on pages 105-115 of "Electron Impact Phenomena and Properties of Gaseous Ions," by F. H. Field and J. L.

5 Franklin (Academic Press, Inc., 1957). Energy sources for such high energy ionizing radiation may be electron accelerators of the Van de Graaff or linear types or cobalt sources or nuclear reactors, etc. The permissible irradiation dosage is from 4 to 40 watt hours per pound of material with a dosage of from 4 to 20 watt hours per pound preferred. This permissible dosage is equivalent to  $3.2 \times 10^6$  to  $32 \times 10^6$  rad.

For some as yet unexplained reason, methacrylates are ineffective in achieving the desired results while both 15 acrylates and dimethacrylates as well as diacrylates are effective.

The most significant data in terms of pointing out the 20 novelty of this invention resides in observations made of the stress at elongations of 200% (200% modulus).

25 These data are summarized as follows in Table 1. All samples contain about 50% by weight of carbon black (commercial material known as "Philblack O," supplied by Phillips Petroleum Co.). Further properties and exact compositions are listed in Tables 2-10. The carbon black is optional. The invention is applicable to any given SBR or Hevea composition, whether filled or unfilled. If desired any conventional filler may be employed to give its usual effects.

The desired compositions were mixed on a cold mill 30 and test slabs of  $6\frac{1}{2}'' \times 6\frac{1}{2}'' \times 0.1''$  were molded in a press for 5 minutes at 260° F. The slabs were then irradiated either in an X-ray machine or by exposure to a beam of 2 million volt electrons obtained from a Van de Graaff accelerator. To prevent undue heating of 35 samples, intermittent exposures were used; the total dosage being controlled by the total time of exposure. Tests on the treated slabs were carried out by using conventional rubber testing equipment.

TABLE 1

Stress (p.s.i.) at 200% Elongation for Composition  
Containing Various Additives

| Base rubber                                                                    | SBR and Philblack O                  |     |       |       | Smoked sheet and Philblack O |       |       |        |       |
|--------------------------------------------------------------------------------|--------------------------------------|-----|-------|-------|------------------------------|-------|-------|--------|-------|
|                                                                                | Radiation dose, watt hours per pound |     |       |       |                              |       |       |        |       |
|                                                                                | 0                                    | 4.3 | 8.6   | 12    | 17.2                         | 0     | 4.3   | 8.6    | 17.2  |
| 200% Modulus                                                                   |                                      |     |       |       |                              |       |       |        |       |
| None (control)                                                                 | 50                                   | 100 | 200   | ----- | 400                          | 40    | 120   | 200    | 400   |
| 2 pts. ethylene diacrylate                                                     | 50                                   | 130 | 250   | ----- | 530                          | ----- | ----- | -----  | ----- |
| 5 pts. ethylene diacrylate                                                     | 50                                   | 240 | 400   | ----- | 750                          | ----- | ----- | -----  | ----- |
| 10 pts. ethylene diacrylate                                                    | 50                                   | 350 | 750   | ----- | 1,200                        | ----- | ----- | -----  | ----- |
| 2 pts. ethylene dimethacrylate                                                 | 50                                   | 170 | 350   | 700   | -----                        | ----- | ----- | -----  | ----- |
| 5 pts. ethylene dimethacrylate                                                 | 50                                   | 240 | 500   | 930   | -----                        | ----- | ----- | -----  | ----- |
| 10 pts. ethylene dimethacrylate                                                | 50                                   | 400 | 750   | 1,400 | 1,40                         | 1,225 | 1,660 | 1,1450 | ----- |
| 20 pts. ethylene dimethacrylate                                                | 50                                   | 400 | 1,000 | 1,800 | -----                        | ----- | ----- | -----  | ----- |
| 10 pts. octyl methacrylate                                                     | 50                                   | 90  | 170   | 380   | 40                           | 80    | 130   | 370    | ----- |
| 20 pts. octyl methacrylate                                                     | 50                                   | 70  | 160   | 300   | 370                          | 50    | 100   | 180    | 250   |
| 10 pts. tetramethylene diacrylate                                              | 40                                   | 570 | 1,400 | ----- | 40                           | 450   | 930   | 1,830  | ----- |
| 2 pts. glyceryl triacrylate <sup>1</sup>                                       | 50                                   | 100 | 150   | 330   | 50                           | 170   | 250   | 500    | ----- |
| 5 pts. glyceryl triacrylate <sup>1</sup>                                       | 100                                  | 170 | 170   | 320   | 50                           | 120   | 250   | 450    | ----- |
| 10 pts. lauryl acrylate <sup>2</sup>                                           | 35                                   | 125 | 500   | 1,030 | 30                           | 200   | 450   | 700    | ----- |
| 20 pts. lauryl acrylate <sup>2</sup>                                           | 20                                   | 80  | 275   | 1,150 | -----                        | ----- | ----- | -----  | ----- |
| 10 pts. polyethylene glycol dimethacrylate, <sup>3</sup> mol. weight about 340 | .30                                  | 160 | 370   | ----- | 630                          | ----- | ----- | -----  | ----- |

<sup>1</sup> Dosages at 0, 4, 8, and 16 weight hours/pound.

<sup>2</sup> 300% modulus with dosages of 0, 4, 10, 20. Control values of modulus are 46, 138, 225, 645 p.s.i.

<sup>3</sup> Commercial material sold as "Monomer MG-1" by Union Carbide and Carbon Co.

ma rays and high speed electrons (e.g., accelerated through 200,000 volts or more) are particularly suitable to this invention. In general, the operative radiation may be described as high energy radiation, the individual particles or photons of which possess energies

70 From these data it may readily be observed that significant results are obtained when the following compounds are employed.

(a) Alkyl acrylates.

(b) Acrylic esters of saturated dihydric alcohols.

- (c) Methacrylic esters of saturated dihydric alcohols.  
 (d) Acrylic and methacrylic esters of polydihydric alcohols.

It was observed that glycetyl triacrylate is not effective so that all polyhydric alcohol esters of acrylic acid may not be generally claimed.

The amount of additive used is in all cases at least  $1\frac{1}{2}$  parts, per 100 parts of rubber. The amount used typically varies with the amount of active component in the compound. There should be at least  $1\frac{1}{2}$  parts of acrylate or methacrylate component per 100 parts of rubber. In the case of ethylene diacrylate, where the acrylate component is about 74% of the molecule, 2 parts of the compound are sufficient, while in the case of octyl acrylate, the compound contains only about 40% acrylate hence at least 4 parts are used. Above about 15 parts of acrylate or methacrylate component per 100 parts of rubber, there is very little increase obtained by adding greater quantities of accelerator. As aforesaid, alkyl monomethacrylates are ineffective while dimethacrylates are effective.

The preferred additives are:

- Alkyl acrylates/alkyl from C<sub>4</sub> to C<sub>12</sub>.  
 Diacrylates and dimethacrylates of polyethylene glycol, 25 having a molecular weight of from about 170 to 1000.  
 Diacrylates and dimethacrylates of ethylene, propylene and tetramethylene glycols.

The following Tables 2 to 10 illustrate the invention in more detail.

TABLE 2  
*SBR With Ethylene Diacrylate and Control*

| Stock No.                                | 1     | 2     | 3     | 4     |
|------------------------------------------|-------|-------|-------|-------|
| SBR 1500                                 | 100   | 100   | 100   | 100   |
| Philblack O                              | 50    | 50    | 50    | 55    |
| Ethylene diacrylate                      | 2     | 5     | 10    |       |
| Tensile strength, lbs./in. <sup>2</sup>  |       |       |       |       |
| 0                                        | 106   | 48    | 37    | 37    |
| 4.3                                      | 466   | 545   | 970   | 1,020 |
| 8.6                                      | 1,170 | 1,210 | 1,600 | 2,000 |
| 17.2                                     | 2,500 | 2,190 | 2,290 | 2,190 |
| Elongation, percent                      |       |       |       |       |
| 0                                        | 440   | 440   | 470   | 560   |
| 4.3                                      | 870   | 780   | 620   | 510   |
| 8.6                                      | 690   | 610   | 540   | 430   |
| 17.2                                     | 590   | 480   | 440   | 300   |
| 200% modulus, lbs./in. <sup>2</sup>      |       |       |       |       |
| 0                                        | 50    | 50    | 50    | 50    |
| 4.3                                      | 100   | 120   | 240   | 350   |
| 8.6                                      | 200   | 250   | 400   | 750   |
| 17.2                                     | 400   | 530   | 750   | 1,200 |
| Durometer                                |       |       |       |       |
| 0                                        | 37    | 35    | 30    | 33    |
| 4.3                                      | 41    | 44    | 50    | 56    |
| 8.6                                      | 47    | 51    | 56    | 68    |
| 17.2                                     | 64    | 58    | 62    | 71    |
| Torsional hysteresis at room temperature |       |       |       |       |
| 0                                        |       |       |       |       |
| 4.3                                      |       |       |       |       |
| 8.6                                      |       |       |       |       |
| 17.2                                     |       |       |       |       |
| Torsional hysteresis at 280° F.          |       |       |       |       |
| 0                                        |       |       |       |       |
| 4.3                                      |       |       |       |       |
| 8.6                                      |       |       |       |       |
| 17.2                                     |       |       |       |       |
| Tensile strength, lbs./in. <sup>2</sup>  |       |       |       |       |
| 0                                        |       |       |       |       |
| 4.3                                      |       |       |       |       |
| 8.6                                      |       |       |       |       |
| 17.2                                     |       |       |       |       |
| Elongation, percent                      |       |       |       |       |
| 0                                        |       |       |       |       |
| 4.3                                      |       |       |       |       |
| 8.6                                      |       |       |       |       |
| 17.2                                     |       |       |       |       |
| 200% modulus, lbs./in. <sup>2</sup>      |       |       |       |       |
| 0                                        |       |       |       |       |
| 4.3                                      |       |       |       |       |
| 8.6                                      |       |       |       |       |
| 17.2                                     |       |       |       |       |
| Durometer                                |       |       |       |       |
| 0                                        |       |       |       |       |
| 4.3                                      |       |       |       |       |
| 8.6                                      |       |       |       |       |
| 17.2                                     |       |       |       |       |

4  
*TABLE 3*  
*SBR With Ethylene Dimethacrylate*

| Stock No.                                | 5     | 6     | 7     | 8     |
|------------------------------------------|-------|-------|-------|-------|
| SBR 1500                                 | 100   | 100   | 100   | 100   |
| Philblack O                              | 50    | 50    | 55    | 60    |
| Ethylene dimethacrylate                  | 2     | 5     | 10    | 20    |
| Tensile strength, lbs./in. <sup>2</sup>  |       |       |       |       |
| 0                                        | 37    | 35    | 39    | 39    |
| 4.3                                      | 519   | 970   | 1,070 | 1,000 |
| 8.6                                      | 1,700 | 1,910 | 2,060 | 1,890 |
| 17.2                                     | 2,620 | 2,530 | 2,410 | 1,910 |
| Elongation, percent                      |       |       |       |       |
| 0                                        | 410   | 510   | 510   | 460   |
| 4.3                                      | 740   | 580   | 490   | 460   |
| 8.6                                      | 570   | 520   | 400   | 320   |
| 17.2                                     | 440   | 370   | 290   | 180   |
| 200% modulus, lbs./in. <sup>2</sup>      |       |       |       |       |
| 0                                        | 50    | 50    | 50    | 50    |
| 4.3                                      | 170   | 240   | 400   | 400   |
| 8.6                                      | 350   | 500   | 750   | 1,000 |
| 17.2                                     | 700   | 930   | 1,400 | 1,800 |
| Durometer                                |       |       |       |       |
| 0                                        | 34    | 32    | 32    | 25    |
| 4.3                                      | 46    | 51    | 56    | 62    |
| 8.6                                      | 55    | 58    | 68    | 77    |
| 17.2                                     | 60    | 65    | 72    | 83    |
| Torsional hysteresis at room temperature |       |       |       |       |
| 0                                        |       |       |       |       |
| 4.3                                      |       |       |       |       |
| 8.6                                      |       |       |       |       |
| 17.2                                     |       |       |       |       |
| Torsional hysteresis at 280° F.          |       |       |       |       |
| 0                                        |       |       |       |       |
| 4.3                                      |       |       |       |       |
| 8.6                                      |       |       |       |       |
| 17.2                                     |       |       |       |       |
| Stock No.                                | 9     | 10    | 11    | 12    |
| SBR 1500                                 | 100   | 100   | 100   | 100   |
| Philblack O                              | 55    | 50    | 55    | 60    |
| Octyl acrylate                           | 10    | 20    |       |       |
| Octyl methacrylate                       |       |       | 10    | 20    |
| Tensile strength, lbs./in. <sup>2</sup>  |       |       |       |       |
| 0                                        | 37    | 38    | 40    | 39    |
| 4.3                                      | 1,310 | 1,350 | 420   | 252   |
| 8.6                                      | 1,910 | 1,870 | 1,180 | 933   |
| 17.2                                     | 2,070 | 1,890 | 2,080 | 1,870 |
| Elongation, percent                      |       |       |       |       |
| 0                                        | 600   | 490   | 450   | 550   |
| 4.3                                      | 650   | 600   | 840   | 940   |
| 8.6                                      | 520   | 390   | 700   | 740   |
| 17.2                                     | 320   | 230   | 600   | 580   |
| 200% modulus, lbs./in. <sup>2</sup>      |       |       |       |       |
| 0                                        | 50    | 50    | 50    | 50    |
| 4.3                                      | 250   | 270   | 90    | 70    |
| 8.6                                      | 450   | 700   | 170   | 160   |
| 17.2                                     | 930   | 1,450 | 380   | 370   |
| Durometer                                |       |       |       |       |
| 0                                        | 25    | 25    | 24    | 23    |
| 4.3                                      | 43    | 44    | 33    | 34    |
| 8.6                                      | 52    | 59    | 46    | 44    |
| 17.2                                     | 59    | 65    | 50    | 52    |

**5**  
TABLE 4—Continued

| Stock No.                                | 9    | 10   | 11   | 12   |
|------------------------------------------|------|------|------|------|
| SBR 1500                                 | 100  | 100  | 100  | 100  |
| Philblack O                              | 55   | 50   | 55   | 60   |
| Octyl acrylate                           | 10   | 20   |      |      |
| Octyl methacrylate                       |      |      | 10   | 20   |
|                                          |      |      |      |      |
| Torsional hysteresis at room temperature |      |      |      |      |
| 0                                        |      |      |      |      |
| 4.3                                      |      | .506 |      |      |
| 8.6                                      | .379 | .399 | .447 | .540 |
| 17.2                                     | .270 | .253 | .352 | .448 |
|                                          |      |      |      |      |
| Torsional hysteresis at 280° F.          |      |      |      |      |
| 0                                        |      |      |      |      |
| 4.3                                      |      |      |      |      |
| 8.6                                      | .194 | .228 |      |      |
| 17.2                                     | .106 | .094 | .174 | .214 |

TABLE 5

*SBR With Acrylate and Methacrylate and Control*  
CURED WITH 12 WATT HR./LB. ELECTRON DOSAGE

|                                        |       |       |       |       |
|----------------------------------------|-------|-------|-------|-------|
| Stock No.                              | 13    | 14    | 15    | 16    |
| SB R 1500                              | 100   | 100   | 100   | 100   |
| Philback O                             | 50    | 60    | 60    | 60    |
| Octyl methacrylate (sample 1)          |       | 20    |       |       |
| Octyl methacrylate (sample 2)          |       |       | 20    |       |
| Octyl acrylate                         |       |       |       | 20    |
| Shore A durometer hardness             | 52    | 50    | 48    | 60    |
| Tensile strength, lb./in. <sup>2</sup> | 1,850 | 1,760 | 1,550 | 2,310 |
| Elongation, percent                    | 590   | 610   | 540   | 270   |
| 200% modulus, lb./in. <sup>2</sup>     | 350   | 300   | 300   | 1,400 |

TABLE 6

SBR With Calcium and Lauryl Acrylates and Control

|                              |       |       |       |       |       |
|------------------------------|-------|-------|-------|-------|-------|
| Stock No.                    | 17    | 18    | 19    | 20    | 21    |
| SBR 1500                     | 100   | 100   | 100   | 100   | 100   |
| Phiblack O                   | 50    | 50    | 50    | 55    | 60    |
| Calcium acrylate             |       | 5     | 10    |       |       |
| Lauryl acrylate              |       |       |       | 10    | 20    |
| 300% modulus                 |       |       |       |       |       |
| Doses:                       |       |       |       |       |       |
| 0                            | 46    | 48    | 41    | 35    | 20    |
| 4                            | 138   | 147   | 165   | 125   | 80    |
| 10                           | 225   | 440   | 380   | 500   | 275   |
| 20                           | 645   | 760   | 1,040 | 1,030 | 1,150 |
| Space A durometer hardness   |       |       |       |       |       |
| 0                            | 40    | 40    | 40    | 30    | 21    |
| 4                            | 42    | 45    | 45    | 36    | 28    |
| 10                           | 48    | 51    | 50    | 57    | 50    |
| 20                           | 53    | 55    | 58    | 55    | 52    |
| Tensile strength, p.s.i.     |       |       |       |       |       |
| 0                            | 56    | 74    | 65    | 63    | 55    |
| 4                            | 234   | 290   | 297   | 373   | 168   |
| 10                           | 764   | 1,070 | 970   | 1,460 | 1,010 |
| 20                           | 1,830 | 1,950 | 1,980 | 2,080 | 1,740 |
| Elongation at break, percent |       |       |       |       |       |
| 0                            | 550   | 480   | 430   | 450   | 600   |
| 4                            | 880   | 850   | 780   | 820   | 850   |
| 10                           | 680   | 700   | 610   | 660   | 730   |
| 20                           | 640   | 600   | 500   | 460   | 410   |

6  
TABLE 7

*Smoked Sheet With Octyl Acrylate and Octyl Methacrylate and Control*

|    |                                          |       |       |       |       |       |
|----|------------------------------------------|-------|-------|-------|-------|-------|
| 5  | Stock No.                                | 22    | 23    | 24    | 25    | 26    |
|    | Rubber SS                                | 100   | 100   | 100   | 100   | 100   |
|    | Philblack O                              | 50    | 55    | 60    | 55    | 60    |
|    | Octyl acrylate                           |       | 10    | 20    |       |       |
|    | Octyl methacrylate                       |       |       |       | 10    | 20    |
| 10 | Tensile strength, lbs./in. <sup>2</sup>  |       |       |       |       |       |
|    | Radiation dose, weight hrs./lb:          |       |       |       |       |       |
|    | 0                                        | 181   | 490   | 427   | 182   | 165   |
|    | 4.3                                      | 912   | 1,560 | 1,840 | 771   | 706   |
|    | 8.6                                      | 1,290 | 1,970 | 2,170 | 1,150 | 1,140 |
|    | 17.2                                     | 1,930 | 2,430 | 2,660 | 1,720 | 1,400 |
| 15 | Elongation, percent                      |       |       |       |       |       |
|    |                                          |       |       |       |       |       |
|    | 0                                        | 790   | 800   | 700   | 720   | 760   |
|    | 4.3                                      | 500   | 500   | 520   | 600   | 580   |
|    | 8.6                                      | 470   | 480   | 470   | 530   | 490   |
|    | 17.2                                     | 440   | 410   | 370   | 470   | 480   |
| 20 | 200% modulus, lbs./in. <sup>2</sup>      |       |       |       |       |       |
|    |                                          |       |       |       |       |       |
|    | 0                                        | 40    | 50    | 60    | 40    | 50    |
|    | 4.3                                      | 120   | 200   | 240   | 80    | 100   |
|    | 8.6                                      | 200   | 370   | 450   | 130   | 180   |
|    | 17.2                                     | 400   | 600   | 930   | 370   | 250   |
| 25 | Durometer                                |       |       |       |       |       |
|    |                                          |       |       |       |       |       |
|    | 0                                        | 25    | 33    | 34    | 24    | 25    |
|    | 4.3                                      | 30    | 40    | 41    | 26    | 30    |
|    | 8.6                                      | 36    | 45    | 50    | 36    | 37    |
|    | 17.2                                     | 45    | 51    | 59    | 43    | 42    |
| 30 | Torsional hysteresis at room temperature |       |       |       |       |       |
|    |                                          |       |       |       |       |       |
|    | 0                                        |       |       |       |       |       |
|    | 4.3                                      |       | .488  | .517  |       |       |
|    | 8.6                                      |       | .339  | .407  | .418  | .481  |
|    | 17.2                                     |       | .266  | .280  | .320  | .340  |
|    |                                          |       |       |       |       |       |
| 35 | Torsional hysteresis at 230° F.          |       |       |       |       |       |
|    |                                          |       |       |       |       |       |
|    | 0                                        |       |       |       |       |       |
|    | 4.3                                      |       |       |       |       |       |
|    | 8.6                                      |       |       |       |       |       |
|    | 17.2                                     |       |       |       |       |       |
| 40 |                                          |       |       |       |       |       |
|    |                                          |       |       |       |       |       |
|    | 0                                        |       |       |       |       |       |
|    | 4.3                                      |       |       |       |       |       |
|    | 8.6                                      |       |       |       |       |       |
|    | 17.2                                     |       |       |       |       |       |
| 45 |                                          |       |       |       |       |       |

TABLE 8

### *Smoked Sheet and SBR With Monomer MG-1 and Tetramethylene Diacrylate*

| Stock No.                               | 27    | 28    | 29    | 30    |
|-----------------------------------------|-------|-------|-------|-------|
| SBR 1500                                | 100   | 100   |       |       |
| Rubber SS                               |       |       | 100   | 100   |
| Philblack O                             | 55    | 55    | 55    | 55    |
| MG-1                                    | 10    |       | 10    |       |
| Tetramethylene diacrylate               |       | 10    |       | 10    |
| Tensile strength, lbs./in. <sup>2</sup> |       |       |       |       |
| Radiation dose, weight hrs./lb.:        |       |       |       |       |
| 0                                       | 38    | 41    | 94    | 145   |
| 4.3                                     | 646   | 1,720 | 1,180 | 1,890 |
| 8.6                                     | 1,800 | 2,030 | 1,740 | 2,150 |
| 17.2                                    | 2,370 | 2,110 | 2,110 | 2,600 |
| Elongation, Percent                     |       |       |       |       |
| 0                                       | 470   | 470   | 840   | 750   |
| 4.3                                     | 670   | 440   | 470   | 390   |
| 8.6                                     | 560   | 230   | 390   | 310   |
| 17.2                                    | 440   | 180   | 340   | 220   |
| 200% modulus, lbs./in. <sup>2</sup>     |       |       |       |       |
| 0                                       | 20    | 40    | 30    | 40    |
| 4.3                                     | 160   | 570   | 200   | 450   |
| 8.6                                     | 370   | 1,400 | 450   | 830   |
| 17.2                                    | 630   |       | 700   | 1,930 |

TABLE 8—Continued

| Stock No.                                | 27   | 28   | 29   | 30   |
|------------------------------------------|------|------|------|------|
| SBR 1500                                 | 100  | 100  | 100  | 100  |
| Rubber SS                                |      |      | 55   | 55   |
| Philblack O                              | 55   | 55   | 55   | 55   |
| MG-1 <sup>1</sup>                        | 10   | 10   | 10   | 10   |
| Tetramethylene diacrylate                |      |      | 10   | 10   |
| Durometer                                |      |      |      |      |
| 0                                        | 23   | 31   | 26   | 24   |
| 4.3                                      | 45   | 56   | 46   | 45   |
| 8.6                                      | 56   | 68   | 56   | 57   |
| 17.2                                     | 61   | 75   | 59   | 65   |
| Torsional hysteresis at room temperature |      |      |      |      |
| 0                                        |      |      |      |      |
| 4.3                                      |      | .424 |      | .460 |
| 8.6                                      | .494 | .324 | .511 | .409 |
| 17.2                                     | .400 | .258 | .439 | .271 |
| Torsional hysteresis at 280° F.          |      |      |      |      |
| 0                                        |      |      |      |      |
| 4.3                                      |      | .183 |      | .287 |
| 8.6                                      | .234 | .104 | .290 | .218 |
| 17.2                                     | .157 | .067 | .215 | .117 |

<sup>1</sup> Dimethacrylate of polyethylene glycol (Carbide and Carbon).

TABLE 9

| Stock No.                                | 31    | 32    | 33    | 34    |
|------------------------------------------|-------|-------|-------|-------|
| Rubber SS                                | 100   | 100   | 100   | 100   |
| SBR 1500                                 |       |       | 50    | 50    |
| Philblack O                              | 50    | 50    | 50    | 50    |
| Glyceryl triacrylate                     | 2     | 5     | 2     | 5     |
| Tensile strength, lbs./in. <sup>2</sup>  |       |       |       |       |
| 0                                        | 430   | 344   | 68    | 69    |
| 4                                        | 1,710 | 1,350 | 480   | 330   |
| 8                                        | 1,620 | 1,740 | 690   | 850   |
| 16                                       | 2,250 | 2,410 | 1,950 | 1,730 |
| Elongation, percent                      |       |       |       |       |
| 0                                        | 700   | 650   | 440   | 520   |
| 4                                        | 490   | 590   | 740   | 820   |
| 8                                        | 490   | 470   | 700   | 650   |
| 16                                       | 430   | 460   | 610   | 580   |
| 200% modulus, lbs./in. <sup>2</sup>      |       |       |       |       |
| 0                                        | 50    | 50    | 50    | 100   |
| 4                                        | 170   | 120   | 100   | 170   |
| 8                                        | 250   | 250   | 150   | 170   |
| 16                                       | 500   | 450   | 330   | 320   |
| Durometer                                |       |       |       |       |
| 0                                        | 35    | 32    | 38    | 36    |
| 4                                        | 41    | 39    | 41    | 42    |
| 8                                        | 42    | 44    | 46    | 48    |
| 16                                       | 48    | 48    | 52    | 51    |
| Torsional hysteresis at room temperature |       |       |       |       |
| 0                                        |       |       |       |       |
| 4                                        | .458  |       |       |       |
| 8                                        | .452  | .402  |       |       |
| 16                                       | .352  | .354  | .424  | .439  |
| Torsional hysteresis at 280° F.          |       |       |       |       |
| 0                                        |       |       |       |       |
| 4                                        |       |       |       |       |
| 8                                        |       |       | .247  |       |
| 16                                       |       | .182  | .179  | .207  |
|                                          |       |       |       | .208  |

TABLE 10

## Pale Crepe With Octyl Acrylate and Control

| Stock No.                  | 35    | 36    |
|----------------------------|-------|-------|
| 5                          | 100   | 100   |
| Pale crepe                 | 50    | 50    |
| Philblack O                |       |       |
| Octyl acrylate             |       | 20    |
| 200% modulus               |       |       |
| 10                         | Dose: |       |
| 0                          | 0     | 60    |
| 4                          | 4     | 140   |
| 10                         | 10    | 310   |
| 20                         | 20    | 575   |
| Tensile strength           |       |       |
| 15                         |       |       |
| 0                          | 0     | 380   |
| 4                          | 4     | 830   |
| 10                         | 10    | 1,660 |
| 20                         | 20    | 2,290 |
| Elongation, percent        |       |       |
| 20                         |       |       |
| 0                          | 0     | 700   |
| 4                          | 4     | 550   |
| 10                         | 10    | 500   |
| 20                         | 20    | 420   |
| Shore A durometer hardness |       |       |
| 30                         |       |       |
| 0                          | 0     | 33    |
| 4                          | 4     | 35    |
| 10                         | 10    | 43    |
| 20                         | 20    | 49    |

In addition to the enhancement of the 200% modulus properties obtained through this invention, tensile strength and torsional hysteresis properties are not adversely affected. For example, irradiation of a sample (Table 3, Stock No. 7) containing 10 parts of ethylene dimethacrylate per 100 parts SBR and 55 parts carbon black at 8.6 watt hours per pound ( $7 \times 10^6$  rad.) yielded a product that developed a stress of 750 p.s.i. at 200% elongation. This should be compared with a comparably exposed sample (Table 2, Stock No. 1), identical in composition except for it not containing any additive. This latter sample developed a stress at 200% elongation of only 200 p.s.i. while non-irradiated samples both with and without additives developed only 50 p.s.i. when stretched to 200% elongation. The enhancement by 275% in its modulus achieved by Stock No. 7 as compared to Stock No. 1 was achieved not only without any reduction in tensile strength but with a 76% increase in tensile strength.

It is to be noted that use of only 2 parts of ethylene dimethacrylate at 17.2 watt hours per pound of ionizing radiation yields a sample (Table 3, Stock No. 5) having a stress at 200% elongation of 700 pounds per square inch, a 175% increase over the value obtained with the comparably exposed additive-free sample while there is an increase of about 5% in the tensile strength observed.

It has been indicated above that the cost of subjecting a material to cure by means of ionizing radiations increases with the amount of radiation necessary. The economical aspect of this invention may be observed by noting that in order to cure an SBR sample sufficiently so as to obtain a 200% modulus of 400 pounds per square inch, an exposure to electrons of 17.2 watt hours per pound is required. Where only 5 parts by weight of ethylene dimethacrylate are premixed with 100 parts of SBR, an exposure of less than 8.6 (probably about 7) watt hours per pound is sufficient to achieve this same result. Thus the cost of irradiation is more than halved through the use of only a minor amount of a relatively inexpensive chemical.

Comparable examples will be noticed in the tables wherein various compounds are shown to have been tested in conjunction with SBR (GR-S), smoked sheet and pale crepe. It has been ascertained that no enhancement is

achieved when these activating compounds of this invention are used in conjunction with neoprene, Paracril, or Butyl rubbers. Some slight enhancement of properties has been obtained with polyethylene and polyvinyl chloride but this enhancement is at best marginal and of little significance.

One sample of 100 parts of smoked sheet containing 55 parts of Philblack O and 10 parts of tetramethylene diacrylate was exposed to X-rays equivalent to 6 watt hours per pound and was observed to have a 200% modulus of 430 pounds per square inch as opposed to a comparably exposed sample containing only 100 parts smoked sheet and 50 parts Philblack O and which gave a 200% modulus value of 230 pounds per square inch. Any other conventional source of ionizing radiation may be substituted for electrons or X-rays, with equivalent results.

Having thus described our invention, what we claim and desire to protect by Letters Patent is:

1. A method of vulcanizing a rubber composition, comprising subjecting said composition to a dosage of from 4 to 40 watt hours of high energy ionizing radiation per pound of said composition, the said composition comprising 100 parts by weight of a rubber selected from the group consisting of Hevea rubber and SBR, and, as an accelerator, from 1.5 to 15 parts of a material selected from the group consisting of alkyl acrylates, acrylic esters of saturated dihydric alcohols, methacrylic esters of saturated dihydric alcohols, acrylic esters of polydihydric alcohols, and methacrylic esters of polydihydric alcohols.

2. A method of vulcanizing a rubber composition, comprising subjecting said composition to a dosage of from 4 to 20 watt hours of high energy ionizing radiation per pound of said composition, the said composition comprising 100 parts by weight of a rubber selected from the group consisting of Hevea rubber and SBR, and, as an accelerator, from 1.5 to 15 parts of a material selected from the group consisting of alkyl acrylates in which the alkyl group has from 4 to 12 carbon atoms, polyethylene glycol diacrylate, polyethylene glycol dimethacrylate, ethylene diacrylate, ethylene dimethacrylate, propylene diacrylate, propylene dimethacrylate, tetramethylene diacrylate, and tetramethylene dimethacrylate, said composition having been vulcanized by the method of claim 1.

3. A method as in claim 2, in which the said accelerator is tetramethylene diacrylate.

4. A method as in claim 2, in which the said accelerator is octyl acrylate.

5. A method as in claim 2, in which the said accelerator is ethylene diacrylate.

6. A vulcanized rubber composition comprising 100 parts by weight of a rubber selected from the group consisting of Hevea rubber and SBR, and, as an accelerator, from 1.5 to 15 parts of a material selected from the group consisting of alkyl acrylates, acrylic esters of saturated dihydric alcohols, methacrylic esters of saturated dihydric alcohols, acrylic esters of polydihydric alcohols and methacrylic esters of polydihydric alcohols, said composition having been vulcanized by the method of claim 1.

7. A vulcanized rubber composition, comprising 100 parts by weight of a rubber selected from the group consisting of Hevea rubber and SBR, and, as an accelerator, from 1.5 to 15 parts of a material selected from the group consisting of alkyl acrylates in which the alkyl group has from 4 to 12 carbon atoms, polyethylene glycol diacrylate, polyethylene glycol dimethacrylate, ethylene diacrylate, ethylene dimethacrylate, propylene diacrylate, propylene dimethacrylate, tetramethylene diacrylate, and tetramethylene dimethacrylate, said composition having been vulcanized by the method of claim 2.

8. A composition as in claim 7, in which the said accelerator is tetramethylene diacrylate.

9. A composition as in claim 7, in which the said accelerator is octyl acrylate.

10. A composition as in claim 7, in which the said accelerator is ethylene diacrylate.

#### References Cited in the file of this patent

#### UNITED STATES PATENTS

|    |           |                |       |               |
|----|-----------|----------------|-------|---------------|
| 30 | 2,155,590 | Garvey         | ----- | Apr. 25, 1939 |
|    | 2,505,067 | Sachs et al.   | ----- | Apr. 25, 1950 |
|    | 2,609,353 | Rubens         | ----- | Sept. 2, 1952 |
|    | 2,668,133 | Brophy et al.  | ----- | Feb. 2, 1954  |
| 35 | 2,670,483 | Brophy         | ----- | Mar. 2, 1954  |
|    | 2,973,309 | Brodney et al. | ----- | Feb. 28, 1961 |

#### FOREIGN PATENTS

|    |         |               |       |               |
|----|---------|---------------|-------|---------------|
| 40 | 546,816 | Belgium       | ----- | Oct. 6, 1956  |
|    | 732,047 | Great Britain | ----- | June 15, 1955 |

#### OTHER REFERENCES

Lawton et al.: "Nature," vol. 172, pp. 76, 77, July 11, 1953.

45 Marans: "Abstracts of Papers of Am. Chem. Soc.," 132nd meeting, page 21T, September 8-13, 1957.

Mesrobian: "Abstracts of Papers of Am. Chem. Soc.," 132nd meeting, page 19Q, September 8-13, 1957.